# EUROPEAN PATENT SPECIFICATION

(11) **EP 0 685 870 B1**
(45) Date of publication and mention of the grant of the patent: **09.09.1998**
(21) Application number: 95108422.7
(22) Date of filing: 01.06.1995
(51) Int. Cl.: H01J 17/00, H01J 9/02, H01J 17/06

(54) **Image display apparatus and method for fabricating the same**
Bildanzeigegerät und Verfahren zur Herstellung desselben
Appareil d'affichage d'image et son procédé de fabrication

(30) Priority: 03.06.1994 JP 122440/94; 13.03.1995 JP 52556/95
(43) Date of publication of application: 06.12.1995
(73) Proprietor: MATSUSHITA ELECTRIC INDUSTRIAL CO., LTD., Kadoma-shi, Osaka 571 (JP)
(72) Inventor: Suzuki, Shigeo, Hirakata-shi, Osaka (JP); Asabe, Mitsuo, Hirakata-shi, Osaka (JP); Shintaku, Hidenobu, Neyagawa-shi, Osaka (JP); Takahashi, Kazuo, Takatsuki-shi, Osaka (JP); Watanabe, Taku, Moriguchi-shi, Osaka (JP); Abe, Yoshiro, Takatsuki-shi, Osaka (JP); Kono, Hiroki, Takatsuki-shi, Osaka (JP); Hirao, Kazunori, Yao-shi, Osaka (JP)
(74) Representative: Kügele, Bernhard

(56) References cited:
- EP-A- 0 450 547
- DE-A- 3 151 101
- PATENT ABSTRACTS OF JAPAN vol. 016, no. 277 (C-0954) 22 June 1992 & JP-A-04 072 057 (SHINKUU YAKIN KK) 06 March 1992

## Description

### 1. Field of the Invention:

The present invention relates to an image display apparatus and a method for fabricating the same; specifically, to an image display apparatus utilizing light emission from a rare gas discharge, which is used for a color television image receptor, a display and the like, and a method for fabricating the same. In particular, the present invention relates to a discharge electrode used in such an image display apparatus and a method for fabricating the same.

### 2. Description of the Reiated Art:

Gas discharge type image display apparatuses such as a plasma display panel (hereinafter, referred to as "PDP") have been utilized as plane type image display apparatuses in information terminal equipment such as a computer. Since the PDPs are advantageous in clear image display and a wide viewing angle as compared with a liquid crystal panel, their application is extended.

As the television image receptor is made larger in size, projection type televisions using a Braun tube and a liquid crystal panel are more and more commercialized. However, such conventional projection type televisions have problems in luminance of the picture and size of the device.

On the other hand, the PDP has drawn attention as an image display device which can be remarkably thinned, Moreover, a technique for obtaining multi-color images in the PDP has been remarkably improved. As a result, the PDP attracts attention as a frontier of the image display device to realize a direct-view type wall-television with high definition. Such a condition requires precise reproducibility and for the life of the PDP to improve.

Figure **20** is a perspective view showing the configuration of a typical DC type PDP **500**.

The DC type PDP **500** includes: a front glass substrate **39** and a rear glass substrate **40** which are made of transparent glass and the like; and a plurality of discharge cells **41** constituted therebetween. A fluorescent material **42** emitting a light beam of a predetermined color is provided inside each of the discharge cells **41**. A gas discharge occurs inside each of the discharge cells **41** so as to generate an ultra-violet ray, and the thus generated ultra-violet ray is radiated onto the fluorescent material **42**, thereby performing a color display.

Specifically, a plurality of cathode lines **43** are formed on the surface of the front glass substrate **39**, which faces the rear glass substrate **40**, so as to be parallel to each other. A plurality of anode lines **44** are formed on the surface of the rear glass substrate **40**, which faces the front glass substrate **39**, so as to be parallel to each other and perpendicularly cross the cathode lines **43**. Each of the cross points of the cathode lines **43** and the anode lines **44** corresponds to a single discharge cell **41**. Each of the discharge cells **41** is separated from another discharge cell **41** by a partition wall **45** and forms a fine discharge tube. The fluorescent materials **42** respectively corresponding to red (R), green (G) and blue (B) are applied onto the respective discharge cells **41** in an appropriate arrangement. The partition wall **45** keeps the distance between the front glass substrate **39** and the rear glass substrate **40** at a predetermined value and prevents the colors of the adjacent discharge cells **41** from being mixed.

An insulating layer **46** is formed on the rear glass substrate **40**. The insulating layer **46** is formed so as to expose the anode lines **44** at positions corresponding to the respective discharge cells **41** and to cover the anode rays **44** in the other region. A cell resistance (not shown in Figure **20**) for limiting the discharge current may be provided for each of the discharge cells **41**.

A discharge gas for radiating an ultra-violet ray is sealed within each of the discharge cells **41**. For example, a mixture of helium and xenon is sealed within the discharge cells **41** so that the gas pressure in the sealed cells **41** can reach about several hundreds Torr.

In the DC type PDP **500** having the above configuration, when a voltage is applied between an arbitrarily selected cathode line **43** and an arbitrarily selected anode line **44**, a discharge occurs in the discharge cell **41** at the position corresponding to the cross point thereof. More specifically, electrons are emitted from the cathode lines **43** to reach the anode lines **44** while ionizing the discharge gas inside the discharge cells **41**. The voltage applied for generating such a discharge is referred to as a writing voltage. The fluorescent materials **42** are excited by the ultra-violet rays generated by the ionization of the discharge gas which attends the discharge, whereby light beams in predetermined colors are emitted in each cell **41**. In this way, a color display is performed.

Figure **21** shows a method for applying a voltage pulse in the case where the DC type PDP **500** shown in Figure **20** is driven by a refresh driving method.

The DC type PDP **500** includes cathode lines **43K1** to **43Kn**, i.e., n cathode lines in total (collectively denoted by the reference numeral **43**) and anode lines **44A1** to **44Am**, i.e., m anode lines in total (collectively denoted by the reference numeral **44**). Each of the cross points of the cathode lines **43** and the anode lines **44** corresponds to each of the discharge cells **41**.

In the refresh driving method, a negative pulse voltage **48** is sequentially applied to the cathode lines **43K1** to **43Kn** in a time-division manner so as to sequentially select the cathode lines **43**. This operation is called scanning, and the cathode lines **43** may be called scanning lines.

Subsequently, the anode lines **44** corresponding to the discharge cells **41** which are expected to emit light beams are selected from the discharge cells **41** along the selected cathode lines **43** in a synchronous manner with the selection of any one of the cathode lines **43**. This selection is performed by applying a positive pulse voltage **51** to the anode lines **44** to be selected. Therefore, if all anode lines **44** are simultaneously selected, all discharge cells **41** on one of the cathode lines **43** are simultaneously selected to emit light. By appropriately selecting the anode lines **44** in accordance with the information to be displayed by the selected cathodes lines **43**, light can be emitted in an arbitrary pattern. In this way, an operation as an image display device is realized.

In the refresh driving method, light-emission occurs only when the writing voltage is applied, and an image is displayed by utilizing the thus emitted light. As the number of cathode lines **43** increases, the time period for a pulse application to each of the cathode lines **43** is shortened. Accordingly, the light-emission time in each of the cathode lines **43** is shortened in inverse proportion to the number of cathode lines **43**. As a result, as the number of cathode lines **43** increases, the luminance of the image to be displayed is lowered.

A memory driving method is used to solve the above problems in the refresh driving method.

Generally, when the discharge occurs in the discharge cells **41** due to application of the writing voltage, charged particles remain in the discharge cells **41**. Owing to these charged particles, even if the application of the writing voltage is stopped, a discharge can be maintained at a lower voltage (Vm) than the initial writing voltage (Vw) over a predetermined time period (normally, several micro seconds). The memory driving method operates the PDP by utilizing this phenomenon.

Figure **22** shows a method for applying a voltage pulse in the case where the DC type PDP 500 shown in Figure **20** is driven by the memory driving method.

Similarly to the refresh driving method, in the memory driving method, a writing voltage **54** of an amplitude Vw is selectively applied to predetermined discharge cells **41** by applying a negative pulse voltage **52** to the cathodes and a positive pulse voltage **53** to the anodes, thereby generating a discharge. In addition, after the application of the writing voltage **54**, a maintaining pulse voltage **55** of an amplitude Vm is subsequently applied to the cathodes so as to prolong the discharge time period.

As described above, in the memory driving method, continuous light emission can be obtained by application of the maintaining pulse voltage **55** regardless of the number of cathode lines. Therefore, the luminance of the image to be displayed can be further enhanced as compared with the refresh driving method utilizing a light emission obtained only by application of the writing voltage. For example, the luminance of 150 cd/m² or more, which is a sufficient value for television display, is accomplished.

The amplitude Vm of the maintaining pulse **55** is required to be set to a voltage Vpd or higher at which the discharge occurs (the discharge cells lighten) in the case where the writing voltage **54** is applied prior to the application of the maintaining voltage **55** and to a voltage Vxt or lower at which the discharge does not occur (the discharge cells do not lighten) in the case where the writing voltage **54** is not applied prior to the application of the maintaining voltage **55**. The difference between these voltages (Vxt - Vpd) is called the memory margin and is generally about 20 V.

In the memory driving method, it is important to obtain a stable discharge voltage for realizing a stable operation of the DC type PDP. The discharge voltage is greatly affected by the cathode lines **43**. Therefore, the cathode lines **43** are very important constituent components in the DC type PDP for reduction in power while the PDP is lightened, long-term stability of operation and reservation of the memory margin.

The cathode lines **43** may be formed of various materials such as metals and oxides. Conventionally, the cathode lines **43** are formed of Ni or an alloy thereof, mainly by screen printing.

Furthermore, a material having a low work function is deposited on the surface of the metal electrodes formed by screen printing in order to reduce the discharge voltage so as to reduce the power consumption of the DC type PDP. For example, Japanese Patent Publication Nos. 2-7136, 5-11381 and 5-11382 disclose such a structure.

Figures **23A** and **23B** schematically show the structure of cathode lines **59** disclosed in Japanese Patent Publication No. 2-7136. Figure **23A** is a cross-sectional view taken along a line **23A-23A'** shown in Figure **23B**.

The cathode line **59** includes a base metal **56** and a porous adhesive layer **57** formed thereon. The base metal **56** is formed into a predetermined pattern (for example, in a stripe pattern in Figure **23B**) by screen printing. The porous adhesive layer **57** made of an oxide or a sulfide of alkaline earth metal elements, or a composite metal oxide of alkaline earth metal elements and aluminum is formed on the base metal **56** by a plasma spraying method in a predetermined pattern corresponding to the arrangement of the discharge cells. In Figure **23B**, the porous adhesive layer **57** is formed in a round shape. At least free alkaline earth metal elements **58** are present in a studded manner inside the pores of the porous adhesive layer **57**.

In such a structure, an electrically insulating material or a material having a high melting point and a low work function is used as an electron-emitting material. By using the electron-emitting material, the discharge voltage is lowered, resulting in reduced power consumption. In the above-mentioned example, the oxide or the sulfide constituting the porous adhesive layer **57** is such a material of a low work function, which serves as the electron-emitting material.

In the case where the porous adhesive layer **57** made of these materials is formed by screen printing, in order that the porous adhesive layers **57** actually function as the cathode lines, it is necessary to perform a melting process and an activating process at a significantly high temperature after forming the porous adhesive layer **57** into a predetermined shape by screen printing, as a step for promoting the generation of free metal elements. On the other hand, in the case where the porous adhesive layer **57** is formed by the plasma spraying method, it is unnecessary to perform a high-temperature process since the plasma spraying step itself is performed at a high temperature. Thus, a cathode line of a low discharge voltage can be formed without applying a large heat load to the glass substrate after depositing the base metal **56** and the porous adhesive layer **57** on the glass substrate.

If the cathode lines are mainly formed by screen printing as described above, the DC type PDP can be fabricated using a relatively simple fabrication device. On the other hand, however, the formation of the cathode lines by screen printing has the following problems.

### (1) Voltage drop due to the line resistance of the cathode lines:

Generally, in the DC type PDP, the cathode lines are sequentially scanned. In this process, if a number of discharge cells on one cathode line are simultaneously selected to be lightened, the current flowing through the discharge flows into the power source via the cathode line. Thus, a difference in voltage due to the line resistance of the cathode line is generated between an end on the power supply side and an end opposite thereto of the cathode line. As a result, as a distance from the power supply side becomes larger, the voltage which is actually applied to the discharge cells is lowered.

In the refresh driving method, this voltage difference appears as a luminance difference. Thus, the quality of the image to be displayed is degraded. In the case of the memory driving method, the memory margin is significantly deteriorated due to the voltage difference.

For example, a discharge current flowing into each discharge cell is about 60 µA, when the electrode pitch is 200 µm, the size of the cathode is 575 µm (length) × 150 µm (width), and He-Xe 10% is sealed, as the discharge gas, within the discharge cell under the pressure of 350 Torr. A sheet resistance of the cathode line having a thickness of 50 µm formed of an aluminum print paste becomes about 40 mΩ. When the DC type PDP having about 900 anodes, which are necessary to an NTSC mode wide television, is constituted under the above conditions, the voltage difference between the power supply side end and the opposite side end of the cathode line is about 6 V. This implies that the memory margin is lowered by about 6 V at the opposite side end as compared with the power supply side end of the cathode line.

In this way, the line resistance bringing about a large voltage drop is one of the reasons for the lowered memory margin.

In the case where the cathode line is formed by screen printing, a metal paste for printing (glass frit) formed by mixing a binder such as a glass powder with a metal powder is generally used. Therefore, when the cathode line is formed by baking the paste which is screen printed into a predetermined patten, the surfaces of metal particles are covered with the melted glass. As a result, the electric conductivity in the cathode line is lowered to about a fraction of that of metal, resulting in an increased line resistance. Therefore, in the cathode lines formed by screen printing, as the screen becomes larger, the line resistance increases because of conspicuous effects of the glass frit. This leads the degree of the voltage drop due to the current flowing through the cathode lines to be large. As a result, the quality of the image to be displayed is degraded, for example, the luminance in a length direction of the cathode line is lowered or some discharge cells are not lightened. In order to solve these problems, a driving voltage circuit is required to be large in scale. Consequently, it is difficult to reduce the fabrication cost or the size.

### (2) Variation in a driving voltage during a lightening time period:

In the memory driving method for driving the PDP within a limited driving voltage range, it is necessary to limit the variation in the driving voltage during the lightening time period to a value as small as possible. However, in the case where, for example, a PDP having aluminum cathodes formed by screen printing is driven by the memory driving method, the driving voltage varies by about 15 V until the driving time period (aging time) reaches 30 thousand hours, for which a television for domestic use should be driven. As a result, the memory margin is remarkably lowered (by -15 V) during the lightening time period. As described above, the surfaces of the cathode lines formed by screen printing are generally covered with glass contained in the paste. As this glass coating is removed by the discharge during the driving, clean metal surfaces gradually appear, thereby varying the driving voltage.

Thus, in order to reduce the line resistance and the variation in the driving voltage during the lightening time period, the cathode lines of the DC type PDP are required to be formed in the state as close as possible to a pure metal.

Although it is also possible to form the cathode lines by vapor deposition, the vapor deposition method has problems in that a formable film is too thin to obtain a predetermined line resistance and the fabrication cost increases since a vacuum vapor deposition apparatus is needed.

In the plasma spraying method, a powdery cathode line material is blown into a jet stream in the high-temperature plasma state to melt the powdery material. The powdery material in the melted state is then adhered to the substrate at a high speed utilizing the energy of the jet stream. Therefore, the glass frit does not basically enter the cathode material, which was a problem in the screen printing method.

However, there is a problem in the process peculiar to the spraying method. In particular, in the case of the spraying utilizing powdery particles of a low specific weight or in the case where a fine pattern is formed over a large area, there arise many problems due to the principle of the spraying method. Therefore, the spraying method cannot be put into practical use as a method for forming the cathode line of the DC type PDP with high accuracy.

Figure **24** schematically shows a method for forming the cathode line by plasma spraying. A glass substrate **60** serving as a front glass substrate of the PDP is directly put on a mounting table **65** made of metal and the like. Cathode line material particles **62** at a high temperature are collided at a high speed against the glass substrate **60** from a plasma spraying torch **61** provided above the glass substrate **60**, thereby forming a thick film made of cathode line material on the surface of the glass substrate **60**. The torch **61** or the substrate **60** is sequentially traversed in a direction indicated by an arrow **64** shown in Figure **24** so as to perform spraying on the entire surface of the glass substrate **60**. In this case, the actual cathode lines **63** are generally formed by using a lift-off method or the like from the thus formed thick film.

In the above conventional plasma spraying method, however, it is difficult to form the cathode lines **63** with a fine pitch and a fine width over the entire surface of the glass substrate **60** without disconnection. Although the glass substrate **60** on which the cathode lines **63** are formed is generally large in size, i.e., about 1 m × 1 m, the thickness thereof is typically small, i.e., about 2 to 3 mm. When the plasma spraying is performed on such a thin and large glass substrate **60**, a difference in temperature occurs between the region where the film deposition is currently being conducted by spraying and the remaining region. The glass substrate **60** may be broken by the thermal stress caused by such a temperature difference. Furthermore, since it is difficult to obtain a uniform thickness over the entire surface of the glass substrate **60**, discharge characteristics may not be uniform. In particular, in the case where the narrow cathode lines **63** are to be formed over a large area using a metal of a small specific weight, it is difficult to attain appropriate characteristics of the cathode lines **63**.

The problem described in the above point (1) similarly occurs in the case where the cathode lines are formed by using a spraying process. This is because, in the case where the cathode line is formed using the spraying process in a conventional method, a bus line (base metal) of the cathode line is formed by screen printing and the surface thereof is covered with the electron-emitting material by a spraying method.

A DC gas discharge type image display apparatus and a method for fabricating the same according to the preambles of claims 17 and 1 repectively are disclosed in DE-A-3151 101.

### SUMMARY OF THE INVENTION

The method for fabricating a DC gas discharge type image display apparatus according to the present invention is defined in claim 1. The DC gas discharge type image display apparatus according to the present invention is defined in claim 17.

In one embodiment, the line electrode included in the set of cathodes are formed on bottom faces of grooves which are formed on a surface of the front glass substrate.

In another embodiment, the spraying method is a plasma spraying method.

In still another embodiment, the cathode material is selected from a group consisting of aluminum, nickel, an aluminum alloy, and a nickel alloy.

In still another embodiment, the discharge gas is a mixed gas of He and Xe.

In still another embodiment, each of the line electrodes included in the line set of cathodes includes : a metal bus line formed by the spraying method ; and an upper coating film made of a material selected from a group consisting of a metal, a metallic oxide, and a metallic sulfide, the upper coating film being formed on a surface of the metal bus line.

In still another embodiment, the upper coating film is formed by the spraying method.

In still another embodiment, the metal bus line is formed by laminating sprayed particles in a flattened manner.

In still another embodiment, the oxide is La₁₋ₓSrₓMO₃ (where M is Co or Mn) having a perovskite structure.

In still another embodiment, each of the line electrodes included in the set of cathodes is formed by laminating sprayed particles of the cathodes material in a flattened manner.

In still another embodiment, the set of cathodes is formed by further being subject to a baking process at a temperature of 400°c or higher after execution of the spraying method.

In still another embodiment, a step of forming the set of cathodes includes the steps of : (a) forming a mask film on the surface of the glass substrate ; (b) forming an opening in a predetermined pattern through the mask film ; (c) depositing a sprayed film serving as the line electrodes included in the set of cathodes at a portion of the surface of the glass substrate, which corresponds to the opening, by spraying a predetermined cathode material from a spraying torch placed above the surface of the mask film and the moving at least one of the spraying torch and the glass substrate ; and (d) removing the mask film form the surface of the glass substrate.

In still another embodiment, the step (c) further includes the step of roughening the portion of the surface of the glass substrate, the portion corresponding to the opening.

In still another embodiment, the step (c) further includes the step of forming the groove having a predetermined depth on the portion of the surface of the glass substrate, the portion corresponding to the opening, and the sprayed film is deposited on a bottom face of the groove.

In still another embodiment, the spraying step is carried out in the step (c) while the glass substrate is placed on a mounting table with a heat insulating means interposed therebetween.

In still another embodiment, a deposition rate of the sprayed film is kept substantially constant with an elapse of a spraying time in the step (c) by controlling either a supply rate of the cathode material form the spraying torch, or a moving rate of at least one of the spraying torch of the glass substrate.

Thus, the invention described herein makes possible the advantages of: (1) providing a DC gas discharge type image display apparatus having a lowresistance cathode line which has a clean metal surface and shows little variation in its driving voltage while driven for a long period of time; and (2) providing a method for fabricating the same.

These and other advantages of the present invention will become apparent to those skilled in the art upon reading and understanding the following detailed description with reference to the accompanying figures.

### BRIEF DESCRIPTION OF THE DRAWINGS

Figure **1** schematically shows a method for producing a cathode line of a DC type PDP in Example 1 according to the present invention.

Figures **2A** to **2F** are cross-sectional views showing the respective fabrication steps of the cathode lines in the PDP in Example 1 according to the present invention.

Figure **3** is a schematic cross-sectional view showing the cathode line formed by Example 1 according to the present invention.

Figure **4** is a graph showing the relationship between the thickness of the cathode line and the resistivity thereof.

Figure **5** is a graph showing a voltage drop in a cathode line in a memory driving method.

Figure **6** is a graph showing the variation in a driving voltage during a long lightening (aging) time period in the memory driving method.

Figures **7A** and **7B** schematically show the change in the shape of material particles to be sprayed due to the execution of a processing step therefor.

Figures **8A** to **8C** schematically show a method for fabricating a cathode line of a DC type PDP in Example 2 according to the present invention.

Figure **9** is a schematic cross-sectional view of a cathode line formed by Example 3 of the present invention.

Figure **10** schematically shows a method for fabricating a cathode line of a DC type PDP in Example 4 according to the present invention.

Figure **11** schematically shows a method for fabricating a cathode line of a DC type PDP in Example 5 according to the present invention.

Figures **12A** to **12F** are cross-sectional views showing the respective fabrication steps of cathode lines in a DC type PDP in Example 6 according to the present invention.

Figure **13A** is a cross-sectional view schematically showing a cathode line formed in a groove in the conventional screen printing, and Figure **13B** is a cross-sectional view schematically showing the cathode line formed in a groove by Example 6 according to the present invention.

Figure **14** is a cross-sectional view schematically showing the shape of a terminal electrode attaching to the cathode line formed by Example 6 according to the present invention.

Figure **15** schematically shows a fabrication process for forming cathode lines on a glass substrate by plasma spraying according to the present invention.

Figure **16** is a graph showing the change in substrate temperatures in the plasma spraying process shown in Figure **15**.

Figure **17** schematically shows a fabrication process for forming cathode lines on a glass substrate by conventional plasma spraying.

Figure **18** is a graph showing the change in substrate temperatures in the conventional plasma spraying process shown in Figure **17**.

Figure **19** is a graph showing the relationships between the substrate temperature, the thickness of a sprayed film, the supply rate of material to be sprayed and the spraying time in the case where cathode lines are formed on a glass substrate by plasma spraying.

Figure **20** is a perspective view showing the configuration of a DC type PDP.

Figure **21** is a diagram showing a refresh driving method of the DC type PDP.

Figure **22** is a diagram showing a memory driving method of the DC type PDP.

Figure **23A** is a cross-sectional view showing the configuration of a cathode line formed by conventional spraying technique, and Figure **23B** is a perspective view of the cathode line shown in Figure **23A**.

Figure **24** is a perspective view schematically showing the process of forming cathode lines on a glass substrate by a spraying method.

### DESCRIPTION OF THE PREFERRED EMBODIMENTS

### Example 1

Figure **1** schematically shows a method for producing a cathode line of a PDP according to a first example of the present invention. Specifically, the cathode line made of metal aluminum is formed on a glass substrate using a plasma spraying method.

A plasma spraying torch **100** includes a water-cooled cathode **1** and a water-cooled anode **2**. A DC voltage is applied between the cathode **1** and the anode **2** by a power source **3** so as to generate an arc discharge **4**. A plasma working gas **5** is supplied from a supply port **5a** thereof which is provided at the rear part of the plasma spraying torch **100**. The supplied plasma working gas **5** is heated and ionized by the arc discharge **4** generated between the cathode **1** and the anode **2** so as to be jetted out of a nozzle **7** as a plasma jet **6**. Argon, helium, hydrogen and the like can be used as the plasma working gas **5**. For example, argon is used in Example 1.

A material **8** to be sprayed which serves as a material of the cathode line is carried by a carrier gas from a supply port **9** in a powdery state so as to be blown into the plasma jet **6**. The material **8** to be sprayed mixes with the plasma jet **6** in the vicinity of a region **X** of Figure **1**, which corresponds to the outside of the nozzle **7**. As a result, the material **8** is heated and melted and then accelerated by the energy of the plasma jet **7** to collide against the surface of a glass substrate **10** at a high speed. With this collision, a coating is formed on the surface of the glass substrate **10**.

The glass substrate **10** functions as a surface glass (front glass) of the image display device (PDP). For example, a soda glass substrate having a thickness of about 2 mm is used as the glass substrate **10**. A mask film **11** having openings **12** corresponding to a pattern of cathode lines **13** to be formed as shown in Figure **1** is attached to the surface of the glass substrate **10**. By performing the spraying from the upper side of the glass substrate **10** through the mask film **11**, the cathode lines **13** having a predetermined thickness are formed only on the portions of the surface of the glass substrate **10**, which correspond to the bottom faces of the openings **12**. By pealing off the mask film **11** after the film deposition by the spraying, the glass substrate **10**, on which the cathode lines **13** are formed into a predetermined pattern, is obtained. The thickness of the mask film **11** is set to about 50 µm, a little thicker than that of the cathode lines to be formed.

The material **8** to be sprayed in Example 1 is metal aluminum powder having a purity of 99%. An average particle size of the powder is about 20 µm.

In the case where an aluminum powder having an average diameter of about 20 µm is blown into the plasma jet **6** as the material **8** to be sprayed, it is desirable for the material **8** to enter into the plasma jet **6** at a small incident angle. In the plasma spraying torch **100** of Figure **1**, in view of structural restrictions thereof, the incident angle θ is set to 30°.

If a plurality of the supply ports **9** of the material **8** are provided in the periphery of the nozzle **7** at equal intervals, the distribution of the plasma jet **6** and the mixing condition of the material **8** therein can be uniform. Therefore, the cathode lines (sprayed film) **13** having better quality can be formed.

The cathode lines (sprayed film) can be formed by arc spraying instead of the plasma spraying. However, in order that the cathode lines having a fine pattern are accurately formed and strongly adhered to the glass substrate, the plasma spaying method is preferred. Moreover, in the plasma spraying method, various materials can be dealt with good controllability.

Figures **2A** to **2F** show the process of forming the cathode lines on the front glass substrate by the plasma spraying method according to the present invention.

First, as shown in Figure **2A**, the mask film **11** is attached onto the surface of the glass substrate **10**. As the mask film **11**, for example, a dry film which is commercially available from TOKYO OHKA KOGYO, Co., Ltd. under the general trade designation "BF series" can be used. Next, as shown in Figure **2B**, openings **12** are formed into a pattern corresponding to the cathode line pattern to be formed on the mask film **11** by an exposing process and an etching process.

Then, as shown in Figure **2C**, blast particles **14** are made to collide against the upper surface of the glass substrate **10** through the mask film **11** on which the openings **12** are formed, thereby conducting a sand blast processing. By this sand blast processing, as shown in Figure **2D**, surfaces **10a** of the portions, which correspond to the openings **12**, of the surface of the substrate **10** are roughened. A preferable surface roughness of the thus obtained rough surface **13a** is typically about 1 in center line average height Ra, although it depends on the material to be sprayed and conditions under which the spraying process is conducted.

Next, as shown in Figure **2E**, the material **8** is made to collide against the surface of the glass substrate **10** by the plasma spraying through the openings **12** formed through the mask film **11**, thereby forming a film made of cathode material. As a result, a sprayed film i.e., a cathode line **13**, is formed on the surface of the glass substrate **10** with strong adhesion corresponding to the openings **12**. On the other hand, the sprayed particles which reach the surface of the mask film **11** recoil due to the elasticity of the mask film **11**. Therefore, the sprayed film **13** is not formed on the surface of the glass substrate **10** other than the portions corresponding to the openings **12**. The mask film **11** is pealed off after the completion of the spraying process, and the cathode lines **13** having a predetermined pattern are formed on the surface of the substrate **10**, as shown in Figure **2F**.

A terminal electrode for connection with an external circuit is further formed on the glass substrate **10**, on which the cathode lines **13** are formed, by the screen printing method. A rear glass substrate formed in another process is then sealed against the glass substrate **10**, thereby obtaining the structure shown in Figure **20**. After creating a vacuum in the gap between the substrates, a mixed gas of He-Xe functioning as a discharge gas is sealed to a predetermined pressure, thereby completing the DC type PDP.

The cathode lines **13** thus formed have the laminated structure of particles as shown in Figure **3**. Specifically, the particles of the sprayed material **8**, which collide in a melted state at a high speed against the surface of the glass substrate **10**, are laminated while being flattened in a horizontal direction (a direction parallel to the surface of the glass substrate **10**), thereby completing the cathode lines **13**. A width W of the cathode lines **13** is typically 150 µm or less, for example, about 100 µm. A thickness h is typically in the range of 10 to 30 µm, for example, about 30 µm.

The surface of the glass substrate **10** is roughened by the sand blast processing in order to increase the adhesion between the cathode lines **13** to be formed and the glass substrate **10**. If the adhesion is not sufficiently strong, the cathode lines **13** may be pealed off or disconnected by a mechanical load acting on the cathode lines **13** due to handling and the like during the fabrication process. As a result, the functions as the cathode lines **13** cannot be reserved in some cases. In particular, in the case where the film made of metal particles is formed on the glass substrate by spraying as in Example 1, difference in thermal expansion between the metal sprayed film (cathode lines) and the glass substrate is large, resulting in small adhesion.

The sand blast processing may be substituted by the following process. Prior to spraying the cathode line material, an extremely thin film is formed by spraying a material exhibiting strong adhesion onto the glass substrate **10**. Thereafter, a predetermined metal material may be sprayed thereon. As such a material capable of functioning as a so-called interlayer, for example, chromium oxide or a material obtained by mixing silica into chromium oxide is considered. Thus, excellent adhesion can be preserved.

Alternatively, in the case where sufficient adhesion can be preserved, such a sand blast processing and a substitution thereof can be completely omitted.

Figure **4** shows the relationship between a resistivity ρ and a thickness h of the cathode lines **13** formed by the plasma spraying method, where a width W of the cathode lines **13** is fixed to be 150 µm. A plot Δ indicates the value in the cathode lines formed by a conventional screen printing method, which is specifically 4.0 × 10⁻⁴ Ω·cm. Each of plots ○ indicates a value in the stage where the cathode lines are formed by the plasma spraying method, and each of plots ● indicates a value after baking is conducted for forming the terminal electrode. The value of a bulk material of the metal aluminum (2.65 × 10⁻⁶ Ω·cm) is also shown in Figure **4**. With respect to the above respective values, the line resistance of the cathode line is measured, respectively. Resistivity values are then obtained by multiplying the measured values by a cross-sectional area of the cathode line (thickness × width) and subsequently dividing the multiplied values by the length.

As is apparent from Figure **4**, although the resistivity in the spraying method decreases as the thickness h increases, it becomes substantially constant at a certain thickness or more. Taking the cathode having a thickness of 30 µm as an example, the resistivity value obtained by spraying is low, i.e., about one-tenth as compared with that obtained by the screen printing method. The difference between the two results from the following. The component of the film formed by the spraying method is mainly a pure aluminum material, except for a small amount of oxide. On the other hand, in the screen printing method, impurities such as glass frit serving as a non-conductive material are inevitably mixed with the metal aluminum material. Therefore, the direct physical contact between aluminum metal particles is inhibited, leading to a lowered conductivity.

The reason why the resistivity decreases as the thickness h increases in the spraying method is regarded as an increase in the probability that particles to be laminated are physically in contact with each other. Although particles having a diameter of 20 µm are used as sprayed particles in the example shown in Figure **4**, the resistivity can be further reduced by using particles having a smaller diameter.

Even in the case where the cathode lines are formed by the plasma spraying method, if the metal aluminum is oxidized in the spraying step, the electrical resistivity of the cathode lines to be formed inevitably increases. In order to prevent the sprayed film from being oxidized, it is sufficient to reduce the pressure of a space (in which a film is formed) leading from the plasma spraying torch to the glass substrate which is subject to spraying during the spraying step.

Next, the effects of the baking process which is performed on the cathode lines formed by the plasma spraying process will be examined. Plots ○ in Figure **4** respectively indicate a resistivity value obtained in the case where the cathode line formed by the plasma spraying is baked at 400°C. At this temperature, i.e., 400°C, the front glass substrate **39** on the cathode side and the rear glass substrate **40** on the anode side are sealed to each other by frit glass in the configuration shown in Figure **20**.

In the cathode lines formed by a plasma spraying method according to the present invention, the resistivity (plots ○) in the stage in which the baking process is not conducted is already about one-tenth of the value of the conventional cathode lines formed by screen printing. In addition, the resistivity after the baking process (plots ●) is further reduced by 30 to 50% as compared with the value before the baking process (plots ○). Simultaneously, the thickness is reduced by about 30 %.

In order to examine the effects of the baking temperature level, the same measurement is performed on another sample which is subject to the similar baking process at a temperature of 580°C. The line resistance after baking the aluminum cathode is reduced to one-third of that before baking. The baking process is carried out in an atmosphere while rising a temperature from room temperature to 580°C in an hour, keeping at 580°C for 10 minutes, and lowering the temperature to room temperature again in an hour.

Regarding the sample baked at 580°C, the cross-section of the sprayed film (cathode line) before and after the baking process is observed with a scanning electron microscope (SEM). As a result, the sprayed film after the baking has a finer laminated structure as compared with that before the baking. It is considered that such a finer laminated structure is obtained because unmelted particles contained in the film immediately after the spraying or particles which are not laminated in the quenching process during the film deposition are melted at a temperature lower than their melting point, that is, a so-called melting point lowering phenomenon occurs.

Furthermore, with respect to the samples which are observed with the SEM, a change in the composition of the sprayed film before and after the baking process is analyzed by an X-ray micro analysis (XMA) method. As a result, the amount of oxygen contained in the sprayed film is slightly reduced after the baking. This signifies that part of aluminum which is oxidized immediately after the spraying is reduced by the baking process. However, the degree of change in the amount of oxygen contained is not large enough to afford a large decrease in the resistivity of the cathode lines. Thus, the resistivity of the cathode lines is considered to be lowered not by reduction of aluminum oxide but mainly by finer quality of sprayed film resulting from baking.

The cathode lines formed by the screen printing method are subject to a similar baking process and a change in the resistivity before and after the process is measured. However, the resistivity of the aluminum cathode lines formed by the screen printing method increases in some cases rather than decreases, after the baking process. Thus, the resistivity thereof is unstable. As described above, the decrease in the resistivity due to the baking process is unique to the cathode lines formed by spraying.

From the above result, it is understood that the resistivity of the cathode line formed by the plasma spraying method is one-tenth of the resistivity of the cathode lines formed by the screen printing method, and can be further reduced to a half thereof or less by the baking process at 400°C or higher in an atmosphere.

Figure **5** shows voltage drops of the cathode lines formed by screen printing and plasma spraying, respectively, in the memory driving method. The dot position (the number of dots) represented by an abscissa corresponds to a size of a screen of the PDP (a length of a cathode line). For example, the number of dots corresponding to a wide television of a 66 cm (26 inch) size is about 900, and that corresponding to a television of 102 cm (40 inch) size is about 1400. The data in Figure **5** is obtained by calculation under condition that a discharge current in each of the discharge cells is 60 µA.

The voltage drops shown in Figure **5** directly represent difference in resistivities of the respective cathode lines. For example, in a 66 cm (26 inch) size television, a voltage drop of 6 V occurs in the cathode fabricated by screen printing. Such a large voltage drop brings about disadvantages such as an extremely wide difference in luminance between the both ends of the screen, decrease in the memory margin, unlighting pixels and the like, which result in deterioration of the quality of the display image. On the other hand, in the cathode fabricated by the plasma spraying method, the voltage drop is small, i.e., about 1 V even in the 66 cm (26 inch) size television. The effect of the voltage drop to such a degree can be sufficiently compensated by the functions of other components. Thus, the same problems as in the screen printing do not occur, and an extremely excellent image can be provided. In the above description, a phenomenon for one cathode line at a certain moment during a driving time period is paid attention to.

The data shown in Figure **5** indicates the result obtained in the case where a driving circuit is provided on one side of the PDP. If driving circuits are provided on both sides of the PDP, a voltage drop in the cathode lines is reduced to, at maximum, a half or less of the data shown in Figure **5**. In consideration of fabrication cost, circuit size and the like, a method for forming the driving circuits on the both sides of the PDP is hardly realizable.

Next, a variation in the driving voltage in the case where the PDP is lightened over a long lightening time period is examined as a long-term life test. The long lightening time period in this case signifies about 30 thousand hours which are generally required as a life of a television for domestic use.

Figure **6** shows the variation in the driving voltage in the case where the DC type PDP is lightened for a long time by the memory driving method. In one PDP, cathode lines in the same panel are separately formed by the screen printing and the plasma spraying. Then, the variation in the driving voltage is measured with respect to each of the cathode lines. Data in Figure 6 are measured in a DC type PDP in which discharge cells having a size of about 300 µm × about 300 µm and a discharge gap of 200 µm of are provided with He - Xe10% gas as a discharge gas sealed at a gas pressure of 350 Torr. Specifically, DC discharges continuously occur with a discharge current of 50 µA for each of the discharge cells. Plots in Figure **6** respectively show average values of the driving voltage for ten pixels dots.

Generally, as the lightening time period elapses, the cathode lines are sputtered by a discharge to be scattered. The scattered particles of the cathode lines attach to the surface of the glass substrate in the periphery of the cathode lines. As a result, in some cases, the cathode area involving the discharge substantially increases, thereby varying the driving voltage. When the data shown in Figure **6** is measured, in order to prevent the discharge area from expanding due to sputtering, a groove pattern is formed on the surface of the glass substrate, and a film made of cathode material is formed on the bottom face of the groove by the screen printing or the plasma spraying, thereby completing the cathode lines.

It can be seen from Figure **6** that, at the time when ten thousand hours elapse from the start of the measurement, the driving voltage is lowered by about 10 V in the cathode line formed by the screen printing. On the other hand, the driving voltage is lowered by about 5 V, that is, a half of the value of the screen printing, in the cathode line formed by the plasma spraying. As the result of continuation of the similar measurement, at the time when 30 thousand hours elapse, the driving voltage of the cathode lines formed by the plasma spraying is lowered by about 8 V, while the driving voltage of the cathode line formed by the screen printing is lowered by about 15 V.

As described above, when the cathode lines are formed by screen printing, it is difficult to drive the PDP in the memory driving method due to the decrease in driving voltage attending the driving for long time. As a result, the function of the PDP as an image display device can be reserved up to about 10 thousand hours at most. On the other hand, when the cathode lines are formed by the plasma spraying method as in the present invention, a high-quality image display can be stably realized while sufficiently reserving the memory margin, in either of the refresh driving method and the memory driving method. These advantages are particularly conspicuous in the latter memory driving method.

In the above description of Example 1, the cathode lines are made of metal aluminum since the metal aluminum is excellent as a cathode line material. This is because metal aluminum is hardly sputtered with respect to the He-Xe mixed gas which is suitable as a discharge gas for realizing a full-color image display.

In the case where a material having a low specific weight and a low melting point such as aluminum is used as a material to be sprayed for forming the cathode lines, as shown in Figure **1**, the structure of the plasma spraying device **100** using a so-called extrapolation mode, in which a spraying powder is blown into the plasma jet 6 after the jetting out thereof, is suitable for forming the cathode lines having excellent properties. In the case where finer particles having a lower specific weight are used, the sprayed material is not sufficiently blown into the plasma jet **6** in some cases. In such cases, there arise problems such as adhesion of the sprayed material in an unmelted state to the surface of the substrate **10** or a decrease in the spraying efficiency.

In order to solve the above problems, it is sufficient to use fine particles which are processed in advance so as to have an appropriate shape. Figures **7A** and **7B** show an example of the change of the particle shape in such a processing process.

Primary particles **16** having an average diameter of d as shown in Figure **7A** are bonded to each other using polyvinyl alcohol (PVA) or the like, thereby forming processed particles **17** each being a set of a plurality of primary particles **16**. As shown in Figure **7B**, each of the processed particles **17** has an average diameter of D (D > d). According to the inventors' experiments, in the case where a 40 kW class plasma spraying apparatus is used, the spraying particles are uniformly blown into the plasma jet 6 by processing the primary particles **16** so that the average diameter **D** of the processed particles **17** is 30 pm or more regardless of the average diameter d of the primary particles **16**, thereby completing a sprayed filn (cathode lines) of good quality. Thus, extremely fine primary particles are also applicable.

Paying attention to the process in which each of the sprayed particles is flattened after colliding against the substrate **10**, in order to obtain a sufficiently fine sprayed film (cathode lines) having sufficiently strong adherence to the glass substrate **10**, it is desirable that the particles being attached to the substrate **10** are flattened so that the diameter of the particles is three times the average diametar d of the primary particles **16**. Furthermore, in order to obtain a fine sprayed film capable of reserving the sufficient adherence to the substrate **10** and reducing the electrical resistivity to the lowest level when the primary particles are flattened as described above so that a sprayed material is adhered to the surface of the glass substrate **10** in such a state that the diameter thereof is about three times the average diameter d of the primary particles **16**, it is desirable that the flattened particles are laminated to three layers or more in a thickness direction of the cathode line, or three flattened particles or more are adhered in a width direction of the cathode line. In the case where the sprayed particles in the sprayed film (cathode lines) are present in such a state, a fine sprayed film (cathode lines) which is most suitable in terms of adherence to the glass substrate and the electrical resistance is formed.

If the average diameter d of the primary particles **16** and the spraying conditions are selected so as to attain the above conditions, a sprayed film, which demonstrates sufficiently good characteristics while being made to function as the cathode lines of the PDP, is formed. Specifically, supposing the formation of cathode lines having a width of W and a thickness of h, by using the spraying powders obtained from the primary particles **16** having an average diameter d which is set in the range, the upper limit thereof being a smaller one of h/2 and W/9 and the lower limit thereof being 10 µm, the cathode lines having a high quality can be formed. A value of 10 µm, which is the lower limit of the average diameter d, is determined, as a minimum value required for efficiently carrying the spraying powder materials in the supply port **9**.

### Example 2

With reference to Figures **8A** to **8C**, Example 2 of the present invention will be described.

The cathode lines **13** formed on the surface of the glass substrate **10** by plasma spraying have, as shown in Figure **8A**, rougher surfaces **13a** as compared with those obtained by screen printing. Therefore, the discharge may concentrate on protrusions of the surfaces **13a** of the cathode lines **13**, thereby eroding a certain portion of the cathode lines **13**.

Thus, in Example 2, in order to eliminating unevenness of the surfaces of the cathode lines **13** formed by plasma spraying, the glass substrate **10** on which the cathode lines **13** are formed is etched by being immersed into an etchant **19** as shown in Figure **8B**. Specifically, the etching is conducted by immersing the glass substrate **10** into the etchant **19** which is a 1.0% sodium hydroxide solution for **15** minutes. Thereafter, the glass substrate **10** taken out of the etchant is washed in flowing water for 10 minutes.

By such an etching process, smoothed surfaces **13b** are provided for the cathode lines **13** as shown in Figure **8C**. Specifically, while an average surface roughness Ra of the surfaces **13a** formed by plasma spraying is about **4**, that of the surfaces **13b** after being subject to the etching process is reduced to about 2. With such a reduced average surface roughness, the discharge is prevented from concentrating on the surfaces of the cathode lines **13**. As a result, the discharge voltage of the PDP can be stabilized over a long-term period.

The surfaces of the cathode lines **13** can be flattened not only by etching utilizing the solution as described above but also by a mechanical process such as grinding.

### Example 3

With reference to Figure **9**, a third example of the present invention will be described.

In the preceding examples, the cathode lines **13** are formed of pure metal (aluminum). When discharge occurs in the cathode lines made of pure metal, there arise problems such as a high discharge voltage, a large sputtering rate and the generation of discharge contraction, although it depends on some conditions such as the kind of discharge gas to be used, the pressure thereof and the configuration of the electrodes.

In order to inhibit the discharge contraction, it is sufficient to constitute the cathode lines by a material of a small sputtering rate, for example, a dielectric material. However, since the dielectric is an insulating material, the cathode lines cannot be formed of dielectric material alone.

Thus, in Example 3, an upper coating **15b** made of dielectric material is formed on bus lines **15a** made of aluminum which is a low resistive metal, thereby constituting cathode lines **15** having a double-layered structure.

Specifically, the bus lines **15a** made of aluminum is first formed by spraying a powder of metal aluminum onto the glass substrate **10** by plasma spraying. At this time, the thickness of the bus line **15a** is typically in the range of 30 to 40 µm. Next, the upper coating **15b** made of a mixture of metal aluminum and dielectric is laminated onto the bus lines **15a** by a spraying method or another method. Finally, the glass substrate **10** is baked at 400°C or more, thereby forming the cathode lines **15**. Although only one upper coating **15b** is formed in Figure **9,** the cathode lines **15** may include more than one laminated coatings.

As described above, the resistivity of cathode lines **15** can be reduced by forming at least bus lines **15a** of the cathode lines **15** by plasma spraying. The material to be used for plasma spraying is not particularly limited to a particular material.

In the case where the upper coating **15b** is formed by plasma spraying, for example, an alumina powder can be used for spraying in Example 3. Alternatively, the upper coating **15b** made of perovskite type oxide, whose structure is represented by La₁₋ₓSrₓMO₃ (where M is Co or Mn) may be formed on the surfaces of the bus lines **15a** by a spraying method or another method. Even in these cases, when at least bus lines **15a** are formed by plasma spraying, the cathode lines **15** containing only a small amount of impurity can be formed.

By forming the cathode lines having a multilayered structure as in Example 3, the resistivity of the cathode lines can be reduced while the discharge contraction can be inhibited. As a result, cathode lines having more excellent characteristics are formed. Thus, a discharge voltage of the PDP can be stabilized over a long time period.

### Example 4

With reference to Figure **10**, Example **4** of the present invention will be described.

Figure **10** schematically shows the formation of cathode lines of a PDP by plasma spraying in Example **4** according to the present invention. A plasma spraying torch **200** used in Example 4 has basically the same configuration and functions as those of the plasma spraying torch **100** in Example 1 of Figure **1**. In Figures **1** and **10**, since like components are denoted by like reference numerals, and therefore the detailed description thereof is herein omitted.

The plasma spraying torch **200** differs from the plasma spraying torch **100** of Example 1 in that a supply port **209** of the powder of the material **8** to be sprayed is placed perpendicularly to the inner wall of the nozzle **7** so that the spraying material **8** is perpendicularly and directly supplied to the plasma jet **6** inside the nozzle **7**. Specifically, the plasma spraying torch **200** has the interpolation type structure.

The interpolation type plasma spraying torch **200** has an advantage that the spraying material is melted without fail as compared with the extrapolation type plasma spraying torch **100** in which the powder of the spraying material **8** is blown into the plasma jet **6** outside the nozzle. However, if the diameter of the supply port **209** is too small or the flow rate of carrier gas is insufficient, the powder of spraying material **8** is melted inside the supply port **209** so as to adhere to the inner wall thereof. In such a case, operational efficiency is lowered, and the quality of film of the cathode lines (sprayed film) **13** is deteriorated due to lumps of the adhered spraying material falling out so as to be supplied onto the glass substrate **10**. Therefore, the diameter of supply port **209** of the spraying material **8** and the flow rate of carrier gas are required to be optimized so as to prevent such disadvantages.

Moreover, in the structure of Figure **10**, the supply port **209** of the spraying material **8** is only unidirectionally provided. On the other hand, if a plurality of supply ports are provided in the periphery of the nozzle **7** at equal angular intervals, the distribution of the plasma jet **6** and a mixing condition of the spraying material therewith are uniformed, thereby forming the cathode lines (sprayed film) **13** of a more excellent quality.

### Example 5

With reference to Figure **11**, Example 5 of the present invention will be described.

Figure **11** schematically shows the formation of cathode lines of a PDP by plasma spraying in Example 5 according to the present invention. A plasma spraying torch **300** used in Example 5 has basically the same configuration and functions as those of the plasma spraying torch **200** in Example 2 of Figure **10**. In Figures **10** and **11**, like components are denoted by like reference numerals, and therefore the detailed description thereof is herein omitted.

The plasma spraying torch **300** of Example 5 differs from the plasma spraying torch **200** of Example 2 in that a casing **317** for controlling the atmosphere is provided below the plasma spraying torch **300**. The casing **317** is provided so as to enclose a space from a lower part of a nozzle outlet **318** of the plasma spraying torch **300** to the vicinity of the upper surface of the glass substrate **10** on which a material is sprayed.

Furthermore, inside the casing **317**, an inert gas **319** is lead from an introducing port **320**. As the inert gas **319**, argon, helium or the like can be used. Alternatively, instead of the inert gas, a reducing gas, for example, gaseous hydrogen and the like may be introduced.

A space **322** is provided between the upper surface of the glass substrate **10** and a lower end **321** of the casing **317**. A gas of the plasma jet **6**, the inert gas **319** introduced, and particles which do not adhere to the glass substrate **10** among the sprayed particles **8** are exhausted outside via the space **322**.

In the case where spraying is performed in a plasma spraying torch without the casing **317**, for example, aluminum is sprayed onto the glass substrate **10** in an atmosphere, the formed sprayed film (cathode lines) **13** is oxidized by oxygen in the atmosphere, which is taken in the plasma jet **6** in the vicinity of the upper surface of the glass substrate **10**. On the other hand, in the plasma spraying torch **300** in Example 5, since the periphery of the plasma jet **6** is enclosed by the casing **317** and the inert gas **319** or the reducing gas is introduced thereto, the sprayed film is not oxidized. Thus, an electrical resistivity is prevented from increasing due to the oxide entering the cathode lines, thereby forming cathode lines having more excellent characteristics.

### Example 6

Figures **12A** to **12F** show another process of forming the cathode lines on the front glass substrate according to the present invention.

First, as shown in Figure **12A**, a mask film **21** is attached onto the surface of the glass substrate **20**. As the mask film **21**, for example, a dry film which is commercially available from TOKYO OHKA KOGYO, Co., Ltd. under the general trade designation "BF series" can be used. Next, as shown in Figure **12B**, openings **22** are formed into a pattern corresponding to a cathode line pattern to be formed on the mask film **21** by an exposing process and an etching process.

Furthermore, as shown in Figure **12C**, blast particles **24** are made to collide against the upper surface of the glass substrate **20** through the mask film **21** on which the openings **22** are formed, thereby conducting a sand blast processing. By this sand blast processing, as shown in Figure **12D**, grooves **25** are formed at the positions corresponding to the openings **22** in the surface of the glass substrate **20**. The sand blast processing forms the grooves **25** as well as roughens the bottom face of the grooves **25**. A preferable degree of the roughening changes depending on the sprayed material, spraying conditions and the like. Typically, it is desirable that a roughened surface whose center line average roughness Ra is about 1. As previously described in connection with the first example, the adherence between the cathode lines to be formed and the glass substrate can be increased by roughening the surface of the glass substrate.

Next, as shown in Figure **12E**, the spraying material **28** is made to collide against the surface of the glass substrate **20** by plasma spraying through the openings **22** provided though the mask film **21**, thereby forming a film made of a cathode line material. As a result, a sprayed film, that is, cathode lines **23**, having strong adherence is formed on the bottom faces of the grooves **25** of the glass substrate **20** corresponding to the openings **22**. On the other hand, the sprayed particles which reach the surface of the mask film **21** recoil due to the elasticity of the mask film **21**. Therefore, the sprayed film **23** is not deposited onto the surface of the glass substrate **20** other than the portions corresponding to the openings **22**. The mask film **21** is pealed off after completion of the spraying process, and then the cathode lines **23** formed only on the bottom faces of the grooves **25** of the substrate **20** are obtained, as shown in Figure **12F**.

As previously described in Example 1, when the PDP is continuously operated over a long lightening time period, for example, about 30 thousand hours, the driving voltage is greatly lowered in the cathode lines formed by conventional screen printing. The increase in the discharge area due to sputtering of the cathode line material is considered as one of the causes of deterioration with aging. On the other hand, if the cathode lines **23** are formed inside the grooves **25** as in Example 6, the increase in the discharge area due to sputtering is inhibited. therefore, variation in the discharge voltage can be inhibited.

However, if the cathode lines are formed inside such grooves **25** by conventional screen printing, the grooves **25** are filled with the cathode material **30** up to the level close to the surface of the substrate **20** in the vicinity of side walls **31** of the grooves **25** as shown in Figure **13A**. Therefore, the cathode line material **30** is scattered outside the grooves **25** by sputtering accompanying the discharge, and the above-mentioned effects are not sufficiently demonstrated.

On the other hand, the sprayed film **23** is formed only on the bottom **29** of the grooves **25** by the plasma spraying method as shown in Figure **13B**. This is because the film formed by spraying utilizes linearly moving particles to be deposited in principle so that the sprayed particles are prevented from adhering to the side walls **31** of the grooves **25**.

Figure **14** is a cross-sectional view schematically showing the structure of the glass substrate **20**, on which the cathode lines **23** are formed in accordance with Example 6, in the vicinity of a terminal electrode **32**.

Since the cathode line **23** is formed on the bottom **29** of the groove **25**, there is a difference in level **33** between the terminal electrode **32** and the cathode line **23** on the glass substrate **20**. Therefore, an electrical connection between the two may not be accomplished.

In order to electrically connect the terminal electrode **32** and the cathode line **23**, a conductive paste material **34** is molded in the region having the difference in level **33** after the spraying process. As the conductive paste material **34**, for example, a nickel paste can be used. After molding the conductive paste material **34**, a baking process is carried out at 580°C, thereby making the molded conductive paste material **34** function as a connection line for connecting the cathode line **23** and the terminal electrode **32**. The baking process is conducted so as to improve the characteristics of the spraying film (cathode lines) **23** as described in Example 1 as well as bake the conductive paste material **34**. Therefore, this process contributes to the improvement of the resistivity value of the cathode line.

Table 1 shows values of voltage drop in a cathode line being continuously lightened for 30 thousand hours in the plane structure, in which the cathode lines are formed on the surface of the glass substrate, and in the groove structure, in which the cathode lines are formed on the bottoms of the grooves, respectively. Moreover, Table 1 shows values in the case where the cathode lines are formed by plasma spraying and in the case where the cathode lines are formed by screen printing in the respective structures described above. The data in Table 1 is measured in a DC type PDP in which discharge cells having a size of about 300 µm × about 300 µm and a discharge gap of 200 µm of are provided with He - Xe10% gas as a discharge gas sealed at a gas pressure of 350 Torr. Specifically, DC discharges continuously occur with a discharge current of 50 µA for each of the discharge cells.

As can be seen from Table 1, the degree of voltage drop of the groove structure is small as compared with that of the plane structure in both cases where the cathode lines are formed by screen printing and by plasma spraying. Furthermore, in the case where the cathode lines of the groove structure is formed by plasma spraying, the minimum value of voltage drop can be obtained. Therefore, in such a case, the deterioration of the driving voltage with aging can be excellently inhibited.

**[Table 1]**

| | Plane structure | Groove structure |
|---|---|---|
| Screen printing | 20 (V) | 15 (V) |
| plasma spraying | 10 (V) | 7 (V) |

### Example 7

With reference to Figures **15** to **19**, a fabrication process of the cathode line by plasma spraying in the present invention will be further described as a seventh example of the present invention.

Figure **15** schematically shows the fabrication process for forming the cathode line on a glass substrate **432** by plasma spraying according to the present invention. Specifically, in Figure **15**, the rectangular glass substrate **423** (fundamentally corresponding to a wide screen) which is subject to the plasma spraying is viewed from the direction perpendicular to the cathode lines to be formed, that is, a latitudinal direction of the glass substrate **432**.

The glass substrate **432** is mounted on a mounting table **433** made of metal and the like via a jig **434**. An air layer **435** having a thickness of about 1 mm is provided between the mounting table **433** and the glass substrate **432**. A plasma spraying torch **436**, from which a plasma jet **437** including spraying particles is provided so as to collide against the glass substrate **432**, is placed above the glass substrate **432**.

Since the glass substrate **432** is generally large in size, the plasma spraying torch **436** is moved at a predetermined speed in accordance with a predetermined pattern so that the entire upper surface of the glass substrate **432** is subject to spraying with the plasma jet **437**, thereby forming the sprayed film, that is, the cathode lines on the entire surface. In the configuration shown in Figure **15**, a number of cathode lines are formed in a direction vertical to Figure **15**. Therefore, the plasma spraying torch **436** is moved in the direction perpendicular to the figure, thereby forming a cathode line for one line. Next, the plasma spraying torch **436** is moved by a predetermined pitch in a direction indicated by an arrow **438** of Figure **15** so as to form a next cathode line with the similar spraying. By repeating these steps, a sprayed film is formed over the entire surface of the glass substrate **432**.

Alternatively, the glass substrate **432** (or the mounting table **433**) may be moved instead of the plasma spraying torch **436** so as to realize the movement of the relatively same pattern as described above.

For comparison, an example of the spraying process in a conventional method will be described with reference to Figures **17** and **18**. Figure **17** shows a rectangular glass substrate **432'** (fundamentally corresponding to a wide screen) to be subject to spraying, which is viewed from the direction perpendicular to the cathode lines to be formed, that is, a latitudinal direction of the glass substrate **432'**. In a conventional method, the glass substrate **432'** which is subject to spraying is directly placed on a mounting table **433'** made of metal because a heat load applied to the glass substrate **432'** by the plasma jet **437'** which is jet out of the plasma spraying torch **436'** should be released to the mounting table **433'** as soon as possible.

Figure **18** is a graph showing temperature variations in the bottom surface of the glass substrate **432'** at points **a'**, **b'** and **c'** in Figure **17**, respectively. An ordinate corresponds to time in which the spraying has -been proceeded, and an abscissa represents a temperature for each point. Specifically, curves **A'**, **B'** and **C'** of Figure **18** show temperature variations at the points **a'**, **b'** and **c'** in Figure **17**, respectively. As is apparent from Figure **18**, the temperature at each point rises as the plasma jet **437'** gets closer to the point because of the movement of the plasma spraying torch **436'**. The maximum temperature is obtained at the time when the plasma jet **437'** passes immediately above the point, and the temperature decreases as the plasma jet **437'** moves away from the point.

A gradient of rise and fall of the above-mentioned temperature profile becomes steeper as the heat moves more rapidly to the mounting table **433'**. Therefore, the difference between the maximum temperature in the bottom face of the substrate (the temperature when the plasma spraying torch positions immediately above the point) and the temperature after the plasma spraying torch **436'** passes the point, that is, **Tgap'** in Figure **18**, becomes extremely large. The wide difference in temperature generates a thermal stress between the region in which a spraying process is being conducted and the other region on the substrate **433'**. The thermal stress acts on the glass substrate **432'**, thereby breaking the glass substrate **432'**.

In such a conventional method, since the heat quickly moves to the mounting table **433'** side, the value of the maximum temperature Tmax in the bottom face of the glass substrate **432'** can be lowered. On the front surface of the glass substrate **432'**, however, there still remains a region where the temperature reaches an extremely high level because of momentary application of a large heat load and poor thermal conductivity of glass. Accordingly, the temperature difference between the front surface and the bottom face of the glass substrate **432'** becomes large. As a result, the thermal pressure may bring about breaking of the glass substrate **432'**.

In Example 7 of the present invention shown in Figure **15**, in order to solve the above-mentioned problems of a conventional method, the components are configured so that a heat load applied to the glass substrate **432** from the plasma spraying torch **436** is not suddenly released to the mounting table **433** side. Specifically, an abrupt change in temperature as in the conventional example is inhibited by providing the thin air layer **435** between the mounting table **433** and the glass substrate **432**.

Figure **16** is a graph showing the change in temperature of the bottom face of the glass substrate **432** at points **a**, **b** and **c** in Figure **15**, respectively. Similarly to Figure **18**, the ordinate corresponds to time in which the spraying has been proceeded, and the abscissa represents the temperature of each point. Specifically, curves **A**, **B** and **C** of Figure **16** show temperature variations at the points **a**, **b** and **c** in Figure **15**, respectively.

As is apparent from Figure **16**, even if distances between the points **a**, **b** and **c** in Figure **15** are equalized to those between the points **a'**, **b'**, and **c'** in Figure **17**, the temperature variation profiles as indicated by the curves **A**, **B** and **C**, respectively, are obtained. As a result, the difference between the maximum temperature on the bottom face of the substrate (temperature at the time when the plasma spraying torch positions immediately above the point) and the temperature after the plasma spraying torch **436** passes the point, that is, **Tgap** in Figure **16** is smaller than the similar temperature difference **Tgap'** in a conventional method. The breaking of the glass substrate **432** due to the temperature difference Tgap does not occur. The temperature difference Tgap is small because the air layer **435** between the glass substrate **432** and the mounting table **433** acts as a heat insulating layer so as to inhibit the heat from rapidly moving to the mounting table **433** side.

The air layer **435** constitutes a closed space between the mounting table **433** and the glass substrate **432**. When an open space is formed, a free convection is generated by the rise in the temperature of the bottom face of the glass substrate **432**. As a result, heat transfer to the mounting table **433** is accelerated, thereby inhibiting heat insulating effects. Even in the case where the closed space is constituted, if the thickness of the air layer **435** is too large, the free convection is generated. As a result, sufficient heat insulating effects cannot be obtained. Therefore, in order to obtain good heat insulating effects, the thickness of the air layer **435** is preferably about 1 mm or less.

Alternatively, other heat insulating means such as a heat insulating board made of a material excellent in heat insulating properties may be provided instead of the air layer **435**.

Next, the effect of accumulation of heat on the glass substrate, which is coherent to the spraying process, will be described.

As can be seen from Figure **16**, as the plasma spraying process proceeds, the maximum temperature on the surface of the glass substrate **432** gradually rises as indicated with a solid line **D** in Figure **16**. This is because heat attendant on spraying is gradually accumulated in the glass substrate **432** due to the heat insulating effect. The rise in temperature of the glass substrate **432** due to the accumulation of heat inevitably changes the surface condition of the glass substrate **432** which is subject to spraying as the film deposition by spraying proceeds.

Figure **19** shows the relationship between the substrate temperature, the thickness of the sprayed film, the supply rate of the material to be sprayed and the elapsed spraying time period in the case where the cathode lines are formed on the glass substrate by plasma spraying. Specifically, the abscissa in Figure **19** represents the position of the cathode line on the glass substrate **432**, which corresponds to an elapsed spraying time. Curves **B** and **E** represent the maximum temperatures on the bottom face of the glass substrate **432** at the respective positions, and curves **C** and **F** represent the thicknesses of sprayed films (cathode lines) to be formed. Curves **A** and **D** show the amounts of supply of the sprayed material from the plasma spraying torch per time unit (i.e., the supply rate of the spraying material). In each of the data, the curves **B**, **C** and **A** in broken lines show the results in the conventional method, and solid lines **E**, **F** and **D** show the results in Example 7 of the present invention, respectively.

In a conventional method, the supply rate of the spraying material from the plasma spraying torch is generally constant as indicated with the curve **A** regardless of elapsed time of the spraying process. The moving rate of the glass substrate or the plasma spraying torch is generally kept constant. On the other hand, the maximum temperature on the glass substrate gradually rises as the spraying time elapses as indicated with the curve **B**. If the supply rate of the spraying material from the plasma spraying torch is constant, the thickness formed by spraying gradually increases as indicated with the curve **C**. This is because the adhering efficiency of metal aluminum particles used as a sprayed material in example 7 increases as the substrate temperature rises. As a result, the sprayed film (cathode lines) cannot be uniformly formed over the entire surface of the glass substrate.

Thus, in Example 7, the supply rate of the spraying material from the plasma spraying torch is gradually decreased as the spraying process elapses as indicated with the curve **D**. Thus, the amount of heat transferred to the glass substrate by the plasma jet gradually decreases, and the maximum temperature of the substrate is inhibited from rising as indicated with the curve **E**. As a result, the thickness of the film formed by the spraying is kept constant as indicated with the curve **F** regardless of the elapse of the spraying process.

As a specific method for reducing the supply rate of the sprayed material from the plasma spraying torch, a method for reducing the output of the plasma jet or a method for reducing the amount of supply of the sprayed material is applicable. Alternatively, when the amount of supply of the sprayed material for a unit area of the glass substrate is relatively reduced by accelerating the moving rate of the plasma spraying torch or the glass substrate, it is also possible to obtain an effect equivalent to that obtained in the case where the supply rate of the spraying material from the plasma spraying torch is gradually reduced. In Example 7, the supply rate of the spraying material is controlled by controlling the moving rate of the plasma spraying torch or the glass substrate, which can be relatively easily realized.

As described above, according to the present invention, cathode lines of a DC gas discharge type image display apparatus are formed by a spraying method. When the cathode lines are formed by a screen printing method which is a conventional method, glass frit (metal paste for printing), which is a non-conductive material, inevitably enters the cathode lines. As a result, the electrical resistivity of the cathode lines increases. On the other hand, the cathode lines formed by the spraying method according to the present invention are mainly constituted by pure metal particles (sprayed particles), except for a small amount of oxide. Therefore, the line resistance thereof is greatly lowered. With the reduced line resistance, in the case where the display apparatus is driven either by a refresh driving method or by a memory driving method, the deterioration of quality of an image, which results from such reasons as uneven luminance of the display screen, unlighted pixels and a reduced memory margin due to a voltage drop along the cathode line, can be prevented. In particular, since the memory margin can be reserved over a long period of time and variation in the driving voltage can be limited to a small value as compared with the method adopting screen printing, the reliability as a display apparatus is remarkably improved.

When grooves are formed into a predetermined pattern on the surface of a front glass substrate and the cathode lines are formed on the bottom faces of the grooves, the constituting material of the cathode lines are not scattered over a large area even in the case where the discharge repeatedly occurs. Therefore, the discharge area is not increased as a discharge time elapses. As a result, a stable operation of a display apparatus can be obtained over a long time period by inhibiting the discharge voltage caused by such an expansion in the discharge area.

When the spraying process is carried out, an average diameter d of a primary particle of the cathode material (spraying material) to be supplied to a spraying apparatus is set so as to be in a certain range, in which the upper limit thereof is a smaller value of h/2 and W/9 and the lower limit thereof is 10 µm, for a width W and a thickness h of the cathode line to be formed. Then, the sprayed particles are adhered to the surface of the glass substrate in such a state that a sprayed particle is flattened so as to have a diameter about three times the average diameter d of the primary particle. As a result, such a fine sprayed film that adhesion with the glass substrate is sufficiently preserved and an electrical resistivity is reduced to an extremely low level can be obtained.

When the plasma spraying is executed as a spraying process, cathode lines having a fine pattern can be formed so as to be minute and to have strong adhesion to the glass substrate. Moreover, in the plasma spraying, a wide variety of materials can be processed with good controllability. Therefore, cathode lines having more excellent characteristics can be formed with high reproducibility.

Moreover, the cathode lines formed in accordance with the present invention may have the structure consisting of a metal bus line and an upper coating formed on the surface thereof. In the cathode lines thus structured, the resistivity of the cathode lines can be reduced by the metal bus line. Simultaneously, the discharge contraction is inhibited by selecting a material having a small sputtering rate as a material for the upper coating.

When a baking process is further carried out after forming the cathode lines by spraying, the sprayed film (cathode lines) is more finely formed, thereby realizing further reduction in the resistivity of the cathode lines.

When the surface of the glass substrate corresponding to the portions where the cathode lines are to be formed is roughened prior to forming the cathode lines by spraying, the adhesion between the sprayed film (cathode lines) and the glass substrate becomes stronger. As a result, even if any mechanical load is applied to the sprayed film, accompanying handling and the like during the fabrication process, problems such as pealing off of the sprayed film (cathode lines) or disconnection thereof do not occur.

When grooves are formed on the surface of the glass substrate corresponding to the portions where the cathode lines are to be formed and the cathode lines are formed on the bottom faces of the grooves by spraying, the material constituting the cathode lines is not scattered over a large area even in the case where the discharge repeatedly occurs. Consequently, the discharge area is not increased as the discharge process elapses. As a result, the operation of the display apparatus is stabilized over a long period of time by inhibiting the discharge voltage from varying due to an expansion in the discharge area (i.e., the area involved in the discharge).

When the spraying process is conducted in such a state that the glass substrate which is subject to spraying is placed on a mounting table via a heat insulating means, the heat which is given to the glass substrate by spraying can be prevented from rapidly transferring to the mounting table. As a result, a temperature difference between the region in which spraying is being conducted and the other region is reduced, thereby reducing a heat load applied to the glass substrate on the surface of the glass substrate. Consequently, the glass substrate is prevented from being broken due to the heat load.

Adhesion efficiency of the sprayed material to the glass substrate gradually increases as the substrate temperature rises. When the deposition rate of the sprayed film is kept substantially constant during the elapse of the spraying time by controlling the supply rate of material to be sprayed from the spraying torch, or the moving rate of at least one of the spraying torch or the glass substrate, the sprayed film (cathode lines) having a substantially uniform thickness can be formed even in the case where the substrate temperature gradually rises due to the accumulation of heat in the glass substrate which is subject to spraying as the spraying time elapses. As a result, even in the case where a large-sized display apparatus is formed, a uniform sprayed film (cathode lines) can be formed over the entire display screen of a large area.

## Claims

1. A method for fabricating a DC gas discharge type image display apparatus (500), comprising :
providing a front glass substrate (10,20,39,432) ;
providing a rear glass substrate (40) facing the front glass substrate, interposing a discharge gas therebetween ;
providing a set of anodes (44) including a plurality of line electrodes formed on the rear glass substrate ;
providing a set of cathodes (13,23,43) including a plurality of line electrodes placed on the front glass substrate so as to perpendicularly cross the set of anodes, wherein the line electrodes included in the set of cathodes are formed by a spraying method for spraying particles (8,28) of a predetermined cathode material from a spraying device (100,200,300,436) toward a glass substrate; and
providing a plurality of discharge cells (41), each being provided so as to correspond to each of cross points of the set of anodes and the set of cathodes;
*characterized* by
selecting said predetermined cathode material so that an average diameter d of a primary particle (16) supplied to the spraying device is set in a range, an upper limit thereof being a smaller value of h/2 and W/9 and a lower limit thereof being 10 µm, where each of the line electrodes included in the set of cathodes has a width W and a thickness h.

2. A method for fabricating a DC gas discharge type image display apparatus according to claim 1, wherein the line electrodes included in the set of cathodes are formed on bottom faces of grooves (25) which are formed on a surface of the front glass substrate.

3. A method for fabricating a DC gas discharge type image display apparatus according to claim 1 or 2, wherein the spraying method is a plasma spraying method.

4. A method for fabricating a DC gas discharge type image display apparatus according to any one of claims 1-3, wherein the cathode material is selected from a group consisting of aluminum, nickel, an aluminum alloy, and a nickel alloy.

5. A method for fabricating a DC gas discharge type image display apparatus according to any one of claims claim 1-4, wherein the discharge gas is a mixed gas of He and Xe.

6. A method for fabricating a DC gas discharge type image display apparatus according to any one of claims 1-5, wherein each of the line electrodes included in the line set of cathodes is provided with :
a metal bus line (15a) formed by the spraying method ; and
an upper coating film (15b) made of a material selected from a group consisting of a metal, a metallic oxide, and a metallic sulfide, the upper coating film being formed on a surface of the metal bus line.

7. A method for fabricating a DC gas discharge type image display apparatus according to claim 6, wherein the upper coating film is formed by the spraying method.

8. A method for fabricating a DC gas discharge type image display apparatus according to claim 6 or 7, wherein the metal bus line is formed by laminating sprayed particles in a flattened manner.

9. A method for fabricating a DC gas discharge type image display apparatus according to any one of claims 6-8, wherein the oxide is La₁₋ₓSrₓMO₃ having a perovskite structure, where M is Co or Mn.

10. A method for fabricating a DC gas discharge type image display apparatus according to any one of claims 1-9, wherein each of the line electrodes included in the set of cathodes is formed by laminating sprayed particles of the cathodes material in a flattened manner.

11. A method for fabricating a DC gas discharge type image display apparatus according to any one of claims 1-10, wherein the set of cathodes is formed by further being subject to a baking process at a temperature of 400°c or higher after execution of the spraying method.

12. A method for fabricating a DC gas discharge type image display apparatus according to any one of claim 1-11, wherein a step of forming the set of cathodes includes the steps of :
(a) forming a mask film (11,21) on the surface of the glass substrate ;
(b) forming an opening (12,22) in a predetermined pattern through the mask film ;
(c) depositing a sprayed film serving as the line electrodes included in the set of cathodes at a portion of the surface of the glass substrate, which corresponds to the opening, by spraying said predetermined cathode material from a spraying torch (100,200,300,436) placed above the surface of the mask film and moving at least one of the spraying torch and the glass substrate ; and
(d) removing the mask film form the surface of the glass substrate.

13. A method for fabricating a DC gas discharge type image display apparatus according to claim 12, wherein the step (c) further includes the step of roughening the portion of the surface of the glass substrate, the portion corresponding to the opening.

14. A method for fabricating a DC gas discharge type image display apparatus according to claim 12 or 13, wherein the step (c) further includes the step of forming the groove (25) having a predetermined depth on the portion of the surface of the glass substrate, the portion corresponding to the opening, and the sprayed film is deposited on a bottom face of the groove.

15. A method for fabricating a DC gas discharge type image display apparatus according to any one of claims 12-14, wherein the spraying step is carried out in the step (c) while the glass substrate is placed on a mounting table (433) with a heat insulating means (435) interposed therebetween.

16. A method for fabricating a DC gas discharge type image display apparatus according to any one of claims 12-15, wherein a deposition rate of the sprayed film is kept substantially constant with an elapse of a spraying time in the step (c) by controlling either a supply rate of the cathode material from the spraying torch, or a moving rate of at least one of the spraying torch or the glass substrate.

17. A DC gas discharge type image display apparatus (500) comprising :
a front glass substrate (10,20,39,432) ;
a rear glass substrate (40) facing the front glass substrate, interposing a discharge gas therebetween ;
a set of anodes (44) including a plurality of line electrodes formed on the rear glass substrate ;
a set of cathodes (13,23,43) including a plurality of line electrodes placed on the front glass substrate so as to perpendicularly cross the set of anodes, wherein the line electrodes included in the set of cathodes are formed by a spraying method for spraying particles (8,28) of a predetermined cathode material from a spraying device (100,200,300,436) toward a glass substrate; and
a plurality of discharge cells (41), each being provided so as to correspond to each of cross points of the set of anodes and the set of cathodes;
*characterized in that*
the cathode material is selected so that an average diameter d of a primary particle (16) supplied to the spraying device is set in a range, an upper limit thereof being a smaller value of h/2 and W/9 and a lower limit thereof being 10 µm, where each of the line electrodes included in the set of cathodes has a width W and a thickness h.

## Patentansprüche

1. Verfahren zur Herstellung eines DC (Gleichstrom)-Gasentladung Bildanzeigegerätes (500) mit den folgenden Schritten:
Bereitstellen eines vorderen Glassubstrats (10, 20, 39, 432);
Bereitstellen eines hinteren Glassubstrats (40), das dem vorderen Glassubstrat zugewandt ist, wobei ein Entladungsgas dazwischen eingebracht wird;
Bereitstellen eines Anodensatzes (44) mit mehreren, auf dem hinteren Glas-substrat ausgebildeten Zeilen- bzw. Linien- bzw. Linearelektroden;
Bereitstellen eines Kathodensatzes (13, 23, 43) mit mehreren Zeilen- bzw. Linien- bzw. Linearelektroden, die auf dem vorderen Glassubstrat so angeordnet sind, daß sie den Anodensatz rechtwinklig kreuzen, wobei die Linearelektroden im Kathodensatz durch ein Sprühverfahren zum Sprühen von Partikeln (8, 28) eines vorbestimmten Kathodenmaterials aus einer Sprühvorrichtung (100, 200, 300, 436) auf ein Glassubstrat ausgebildet werden; und
Bereitstellen mehrerer Entladungszellen (41), von denen jede so vorgesehen ist, daß sie mit jedem Kreuzungspunkt des Anodensatzes und des Kathodensatzes übereinstimmt;
**gekennzeichnet durch**
eine solche Auswahl des vorbestimmten Kathodenmaterials, daß der mittlere Durchmesser d eines Primärpartikels (16), der der Sprühvorrichtung zugeführt wird, in einem Bereich eingestellt wird, dessen obere Grenze ein kleinerer Wert von h/2 und W/9 ist und dessen untere Grenze 10 µm ist, wobei jede der Linearelektroden, die im Kathodensatz enthalten sind, eine Breite W und eine Dicke h hat.

2. Verfahren zur Herstellung eines DC (Gleichstrom)-Gasentladung-Bildanzeigegerätes nach Anspruch 1, bei dem die Linearelektroden, die im Kathodensatz enthalten sind, auf Bodenflächen von Rillen (25) ausgebildet sind, welche auf einer Oberfläche des vorderen Glassubstrats ausgebildet sind.

3. Verfahren zur Herstellung eines DC (Gleichstrom)-Gasentladung-Bildanzeigegerätes nach Anspruch 1 oder 2, bei dem das Sprühverfahren ein Plasmasprühverfahren ist.

4. Verfahren zur Herstellung eines DC (Gleichstrom)-Gasentladung-Bildanzeigegerätes nach einem der Ansprüche 1 bis 3, bei dem das Kathodenmaterial aus einer Gruppe ausgewählt wird, die aus Aluminium, Nickel, einer Aluminiumlegierung und einer Nickellegierung besteht.

5. Verfahren zur Herstellung eines DC (Gleichstrom)-Gasentladung-Bildanzeigegerätes nach einem der Ansprüche 1 bis 4, bei dem das Entladungsgas ein Gasgemisch aus He und Xe ist.

6. Verfahren zur Herstellung eines DC (Gleichstrom)-Gasentladung-Bildanzeigegerätes nach einem der Ansprüche 1 bis 5, bei dem jede der Linearelektroden im linearen Kathodensatz versehen ist mit:
einer Metall-Busleitung (15a), die durch das Sprühverfahren ausgebildet wird, und
einem oberen Beschichtungsfilm (15b), der aus einem Material hergestellt ist, das aus einer Gruppe ausgewählt wird, die aus einem Metall, aus einem metallischen Oxid und einem metallischen Sulfid besteht, wobei der obere Beschichtungsfilm auf einer Oberfläche der Metall-Busleitung ausgebildet ist.

7. Verfahren zur Herstellung eines DC (Gleichstrom)-Gasentladung-Bildanzeigegerätes nach Anspruch 6, bei dem der obere Beschichtungsfilm durch das Sprühverfahren ausgebildet wird.

8. Verfahren zur Herstellung eines DC (Gleichstrom)-Gasentladung-Bildanzeigegerätes nach Anspruch 6 oder 7, bei dem die metallische Busleitung durch das Laminieren gesprühter Partikel in abgeflachter Weise ausgebildet wird.

9. Verfahren zur Herstellung eines DC (Gleichstrom)-Gasentladung-Bildanzeigegerätes nach einem der Ansprüche 6 bis 8, bei dem das Oxid La₁₋ₓSrₓMO₃ mit einer Perovskit-Struktur ist, wobei M Co oder Mn ist.

10. Verfahren zur Herstellung eines DC (Gleichstrom)-Gasentladung-Bildanzeigegerätes nach einem der Ansprüche 1 bis 9, bei dem jede der Linearelektroden im Kathodensatz durch das Laminieren gesprühter Partikel des Kathodenmaterials in abgeflachter Weise ausgebildet wird.

11. Verfahren zur Herstellung eines DC (Gleichstrom)-Gasentladung-Bildanzeigegerätes nach einem der Ansprüche 1 bis 10, bei dem der Kathodensatz dadurch ausgebildet wird, daß er nach dem Durchführen des Sprühverfahrens ferner einem Backverfahren bei einer Temperatur von 400°C oder höher unterzogen wird.

12. Verfahren zur Herstellung eines DC (Gleichstrom)-Gasentladung-Bildanzeigegerätes nach einem der Ansprüche 1 bis 11, bei dem die Ausbildung des Kathodensatzes die folgenden Schritte aufweist:
(a) Ausbilden eines Maskenfilms (11, 21) auf der Oberfläche des Glassubstrats;
(b) Ausbilden einer Öffnung (12, 22) in einem vorbestimmten Muster durch den Maskenfilm;
(c) Ablagern eines Sprühfilms, der als im Kathodensatz enthaltene Linearelektroden dient, an einem Abschnitt der Oberfläche des Glassubstrats, welcher der Öffnung entspricht, durch das Sprühen des vorbestimmten Kathodenmaterials aus einem Sprühbrenner (100, 200, 300, 436), der über der Oberfläche des Maskenfilms angeordnet ist, und Bewegen des Sprühbrenners und/oder des Glassubstrats; und
(d) Entfernen des Maskenfilms von der Oberfläche des Glassubstrats.

13. Verfahren zur Herstellung eines DC (Gleichstrom)-Gasentladung-Bildanzeigegerätes nach Anspruch 12, bei der der Schritt (c) ferner den Schritt des Aufrauhens des Abschnittes der Oberfläche des Glassubstrats beinhaltet, der der Öffnung entspricht.

14. Verfahren zur Herstellung eines DC (Gleichstrom)-Gasentladung-Bildanzeigegerätes nach Anspruch 12 oder 13, bei dem der Schritt (c) ferner den Schritt des Ausbildens der Rille (25) mit einer vorbestimmten Tiefe auf dem Abschnitt der Oberfläche des Glassubstrats umfaßt, der der Öffnung entspricht, wobei der Sprühfilm auf einer Bodenfläche der Rille abgelagert wird.

15. Verfahren zur Herstellung eines DC (Gleichstrom)-Gasentladung-Bildanzeigegerätes nach einem der Ansprüche 12 bis 14, bei dem der Sprühschritt im Schritt (c) ausgeführt wird, während das Gassubstrat auf einem Befestigungstisch (433) angeordnet ist, wobei dazwischen eine Wärmeisolationseinrichtung (435) angeordnet ist.

16. Verfahren zur Herstellung eines DC (Gleichstrom)-Gasentladung-Bildanzeigegerätes nach einem der Ansprüche 12 bis 15, bei dem die Ablagerungsrate für den Sprühfilm im wesentlichen über den Ablauf der Sprühzeit im Schritt (c) konstant gehalten wird, und zwar durch das Einregeln entweder der Zuführungsrate des Kathodenmaterials aus dem Sprühbrenner oder der Bewegungsrate des Sprühbrenners und/oder des Glassubstrats.

17. DC (Gleichstrom)-Gasentladung-Bildanzeigegerät (500) mit:
einem vorderen Glassubstrat (10, 20, 39, 432);
einem hinteren Glassubstrat (40), das dem vorderen Glassubstrat zugewandt ist, wobei ein Entladungsgas dazwischen eingebracht ist;
einem Anodensatz (44) mit mehreren Zeilen- bzw. Linien- bzw. Linearelektroden, die auf dem hinteren Glassubstrat ausgebildet sind;
einem Kathodensatz (13, 23, 43) mit mehreren Zeilen- bzw. Linien- bzw. Linearelektroden, die auf dem vorderen Glassubstrat so angeordnet sind, daß sie den Anodensatz rechtwinklig kreuzen, wobei die Linearelektroden im Kathodensatz durch ein Sprühverfahren zum Sprühen von Partikeln (8, 28) eines vorbestimmten Kathodenmaterials aus einer Sprühvorrichtung (100, 200, 300, 436) auf ein Glassubstrat ausgebildet werden; und mit
mehreren Entladungszellen (41), von denen jede so vorgesehen ist, daß sie mit jedem Kreuzungspunkt des Anodensatzes und des Kathodensatzes übereinstimmt ;
**dadurch gekennzeichnet,** daß
das Kathodenmaterial so ausgewählt wird, daß der mittlere Durchmesser d eines Primärpartikels (16), der der Sprühvorrichtung zugeführt wird, in einem Bereich eingestellt wird, dessen obere Grenze ein kleinerer Wert von h/2 und W/9 ist und dessen untere Grenze 10 µm ist, wobei jede der im Kathodensatz enthaltenen Linearelektroden eine Breite W und eine Dicke h hat.

## Revendications

1. Procédé pour fabriquer un dispositif (500) de visualisation d'images à courant continu, fonctionnant par décharges dans un gaz, consistant à :
réaliser un substrat en verre avant (10, 20, 39, 432);
réaliser un substrat en verre arrière (40) faisant face au substrat en verre avant, à introduire un gaz pour décharge entre les deux;
réaliser un ensemble d'anodes (44) comprenant une pluralité d'électrodes linéaires formées sur le substrat en verre arrière;
réaliser un ensemble de cathodes (13, 23, 43) comprenant une pluralité d'électrodes linéaires, disposées sur le substrat en verre avant de manière à croiser perpendiculairement l'ensemble d'anodes, les électrodes linéaires faisant partie de l'ensemble des cathodes étant formées par un procédé de projection permettant de projeter des particules (8, 28) d'un matériau cathodique prédéterminé à partir d'un dispositif de projection (100, 200, 300, 436), sur un substrat en verre;
et à réaliser une pluralité de cellules à décharge (41), chacune étant réalisée de manière à correspondre à chacun des points de croisement de l'ensemble d'anodes et de l'ensemble de cathodes;
*caractérisé en ce que*
le matériau cathodique prédéterminé est choisi de manière à ce que le diamètre moyen d d'une particule primaire (16) fournie au dispositif de projection se situe dans une plage ayant comme limite supérieure la plus petite d'entre les deux valeurs h/2 et W/9 et comme limite inférieure 10 µm, chacune des électrodes linéaires de l'ensemble des cathodes ayant une largeur W et une épaisseur h.

2. Procédé pour fabriquer un dispositif de visualisation d'images à courant continu, fonctionnant par décharges dans un gaz, selon la revendication 1, dans lequel les électrodes linéaires faisant partie de l'ensemble de cathodes sont formées sur les faces inférieures de rainures (25), qui ont été formées sur une surface du substrat en verre avant.

3. Procédé pour fabriquer un dispositif de visualisation d'images à courant continu, fonctionnant par décharges dans un gaz, selon la revendication 1 ou 2, dans lequel le procédé de projection utilisé est un procédé de projection par plasma.

4. Procédé pour fabriquer un dispositif de visualisation d'images à courant continu, fonctionnant par décharges dans un gaz, selon l'une quelconque des revendications 1 - 3, dans lequel le matériau des cathodes est choisi dans le groupe constitué par l'aluminium, le nickel, un alliage d'aluminium et un alliage de nickel.

5. Procédé pour fabriquer un dispositif de visualisation d'images à courant continu, fonctionnant par décharge dans un gaz, selon l'une quelconque des revendications 1 - 4, dans lequel le gaz pour décharges est un mélange des gaz He et Xe.

6. Procédé pour fabriquer un dispositif de visualisation d'images à courant continu, fonctionnant par décharges dans un gaz, selon l'une quelconque des revendications 1 - 5, dans lequel chacune des électrodes linéaires faisant partie de l'ensemble de cathodes comprend :
une ligne bus en métal (15a) formée par le procédé de projection; et
un film de revêtement supérieur (15b) réalisé en un matériau choisi dans un groupe constitué par les métaux, les oxydes de métaux, les sulfures de métaux, le film de revêtement supérieur étant formé sur une surface de la ligne de bus en métal.

7. Procédé pour fabriquer un dispositif de visualisation d'images à courant continu, fonctionnant par décharges dans un gaz, selon la revendication 6, dans lequel le film de revêtement supérieur est formé par le procédé de projection.

8. Procédé pour fabriquer un dispositif de visualisation d'images à courant continu, fonctionnant par décharges dans un gaz, selon l'une des revendications 6 ou 7, dans lequel la ligne de bus en métal est formée en stratifiant les particules projetées de manière à être aplaties.

9. Procédé pour fabriquer un dispositif de visualisation d'images à courant continu, fonctionnant par décharges dans un gaz, selon l'une quelconque des revendications 6 - 8, dans lequel l'oxyde est La₁₋ₓSrₓMOₓ, ayant une structure de pérovskite, où M est Co ou Mn.

10. Procédé pour fabriquer un dispositif de visualisation d'images à courant continu, fonctionnant par décharges dans un gaz, selon l'une quelconque des revendications 1 - 9, dans lequel chacune des électrodes linéaires faisant partie de l'ensemble de cathodes est formée en stratifiant les particules du matériau cathodique projetées de manière à être aplaties.

11. Procédé pour fabriquer un dispositif de visualisation d'images à courant continu par décharges dans un gaz, selon l'une quelconque des revendications 1 - 10, dans lequel l'ensemble de cathodes est formé en étant en outre soumis à une opération de cuisson à une température de 400 °C ou plus, après l'exécution du procédé de projection.

12. Procédé pour fabriquer un dispositif de visualisation d'images à courant continu, fonctionnant par décharges dans un gaz, selon l'une quelconque des revendications 1 - 11, dans lequel la formation de l'ensemble de cathodes comprend les étapes consistant à :
(a) former un film constituant un masque (11, 21) sur la surface du substrat en verre;
(b) former une ouverture (12, 22) suivant un motif prédéterminé à travers le film constituant un masque;
(c) déposer un film de particules projetées servant d'électrodes linéaires faisant partie de l'ensemble de cathodes dans une portion de la surface du substrat en verre, qui correspond à l'ouverture, en projetant ledit matériau de cathode prédéterminé, à l'aide d'une torche de projection (100, 200, 300, 436) placée au-dessus de la surface du film servant de masque et en déplaçant la torche de projection et/ou le substrat en verre; et
(d) à enlever le film servant de masque de la surface du substrat en verre.

13. Procédé pour fabriquer un dispositif de visualisation d'images à courant continu, fonctionnant par décharges dans un gaz selon la revendication 12, dans lequel l'étape (c) comprend en plus un traitement visant à rendre rugueuse une portion de la surface du substrat en verre, la portion correspondant à l'ouverture.

14. Procédé pour fabriquer un dispositif de visualisation d'images à courant continu, fonctionnant par décharges dans un gaz, selon la revendication 12 ou la revendication 13, dans lequel l'étape (c) comprend en outre une phase consistant à former une rainure (25) ayant une profondeur prédéterminée sur la portion de la surface du substrat en verre, la portion correspondant à l'ouverture, et le film de particules projetées est déposé sur la face inférieure de la rainure.

15. Procédé pour fabriquer un dispositif de visualisation d'images à courant continu, fonctionnant par décharges dans un gaz, selon l'une quelconque des revendications 12 - 14, dans lequel l'étape de projection se fait à l'étape (c) pendant que le substrat en verre est placé sur une table de travail (433) avec un moyen thermiquement isolant (435) disposé entre les deux.

16. Procédé pour fabriquer un dispositif de visualisation d'images à courant continu, fonctionnant par décharges dans un gaz, selon l'une quelconque des revendications 12 - 15, dans lequel la vitesse de formation du film de particules projetées est maintenue sensiblement constante au cours de la projection à l'étape (c), en contrôlant soit la vitesse d'apport du matériau cathodique depuis la torche de projection, soit la vitesse de déplacement de la torche de projection et/ou du substrat en verre.

17. Appareil (500) de visualisation d'images à courant continu, fonctionnant par décharges dans un gaz, comprenant :
un substrat en verre avant (10, 20, 39, 432);
un substrat en verre arrière (40) faisant face au substrat en verre avant, un gaz pour décharge étant disposé entre les deux;
un ensemble d'anodes (44) comprenant une pluralité d'électrodes linéaires formées sur le substrat en verre arrière;
un ensemble de cathodes (13, 23, 43) comprenant une pluralité d'électrodes linéaires placées sur le substrat en verre avant de manière à croiser perpendiculairement l'ensemble d'anodes,
dans lequel les électrodes linéaires faisant partie de l'ensemble des cathodes sont formées par un procédé de projection permettant de projeter des particules (8, 28) d'un matériau cathodique prédéterminé à partir d'un dispositif de projection (100, 200, 300, 436) sur un substrat en verre;
et une pluralité de cellules à décharges (41), chacune étant réalisée de manière à correspondre à chacun des points de croisement de l'ensemble d'anodes et de l'ensemble de cathodes;
*caractérisé en ce que*
le matériau cathodique est choisi de manière à ce que le diamètre moyen d d'une particule primaire (16) fournie au dispositif de projection se situe dans une plage ayant comme limite supérieure la plus petite d'entre les deux valeurs h/2 et W/9 et comme limite inférieure 10 µm, chacune des électrodes linéaires de l'ensemble des cathodes ayant une largeur W et une épaisseur h.
